

Oct. 21, 1930.

W. C. CALVERT

1,779,388

METHOD OF COATING FABRICS AND PRODUCTS DERIVED THEREFROM

Filed Dec. 2, 1927



Inventor  
William C. Calvert

20y

P. D. Ferguson

Attorney

## UNITED STATES PATENT OFFICE

WILLIAM C. CALVERT, OF EVANSTON, ILLINOIS, ASSIGNOR TO THE GOODYEAR TIRE & RUBBER COMPANY, OF AKRON, OHIO, A CORPORATION OF OHIO

## METHOD OF COATING FABRICS AND PRODUCTS DERIVED THEREFROM

Application filed December 2, 1927. Serial No. 237,341.

My invention relates to the coating of fabrics and it has particular relation to a method of coating fabrics employed in the construction of balloons and breather bags or fabrics of a similar nature.

More specifically, my invention has for one of its objects the provision of a fabric which may be employed in the construction of gas containers for balloons, which is relatively flexible and durable. The fabric also possesses a relatively high resistance to the diffusion of inflating gas through the coating film and yet is comparatively inexpensive to manufacture.

Heretofore, it has been practically universal practice to construct gas containers for balloons of fabric coated either with a film of rubber or with gold beater's skin. The first mentioned material is relatively inexpensive to manufacture, because rubber in the form of a cement is inexpensive and may be readily spread over the surface of the fabric by means of suitable calendering rollers. However, fabric so prepared has a relatively high degree of permeability and an excessive amount of inflating gas (hydrogen or helium) is lost by diffusion of the gas through the coating film. Fabrics coated with gold beater's skin are, in many respects, more satisfactory than rubber coated fabric, because such fabrics have a very high resistance to the diffusion of the inflating gas and are also quite durable and flexible. Since this material (an animal membrane) is obtained only in small pieces hardly more than six or eight inches square its initial cost is not only relatively great, but the proper trimming of the small pieces and the application thereof to extensive surfaces as of gas cells, involves a tedious and expensive process. The cost of fabrics coated with this material is, therefore, so excessive as to preclude their use in any except the most expensive and elaborate of balloons.

Numerous attempts have been made to develop a coating material having the advantages of a rubber coating and also having the durability and the resistance to diffusion of inflating gases characteristic of fabrics coated with gold beater's skin. Dur-

ing the course of these experiments various materials have been suggested and tried, among which specific reference may be made to the cellulose derivatives, such as cellulose acetate, cellulose nitrate, cellulose xanthate, and proteinous materials, such as gelatin. Heretofore, none of these materials has proved to be entirely satisfactory, either because of a lack of flexibility or because of the impossibility of so applying to the fabric as to provide a tenaciously adhering, permanent coating.

This invention consists in the discovery of a novel method of application whereby the materials previously referred to may be caused to adhere readily and permanently to a fabric surface. For a better understanding of the invention, reference may now be had to the single figure of the accompanying drawing, forming a part of the specification and which is a cross-sectional view of a portion of fabric prepared in accordance with the provisions of this invention. The method of application varies somewhat, depending upon the nature of the fabric surface to which the coating is to be applied. For example, to apply a coating of impermeable material to an ordinary rubberized fabric it is necessary, first, to coat the fabric with a rubber suspension, such as latex or rubber cement. Additional coatings containing gelatin or glue, or other adhesive, which will readily adhere to the coating material, are then applied to the surface of the first coating and the gas resistant film is then applied to the latter coating.

The exact course of procedure may be varied, depending upon the character and quality of the product desired. The following is a specific example of a procedure whereby a high grade fabric, particularly adapted for the construction of gas cells for lighter-than-aircraft, is obtained from an ordinary rubber coated fabric.

The fabric 5 is first coated with a layer 6 comprising a solution consisting of approximately 200 cc. of 60 percent latex, or its equivalent, and 1000 cc. of water. A second coating 7 consisting of approximately 100 cc. of 60 percent latex, 30 grams of gelatin, 60 grams

of glycerine and 1000 cc. of water is applied to the first coating. A third coating 8 in which the proportion of latex is relatively decreased while the proportion of gelatin is proportionately increased, consisting of 50 cc. of 5 60 percent latex, 60 grams of gelatin, 120 grams of glycerine and 1000 cc. of water, is next spread over the second coating. This layer is followed by one or more (usually two 10 or three) coats of a solution constituting a layer 9 and consisting of 40 grams of gelatin, 80 grams of glycerine and 1000 cc. of water, in which 2.4 grams of alum (a tanning agent) has been dissolved. This solution is spread 15 upon the fabric and is permitted to dry, preferably while the fabric is stretched upon a table or upon a tentering frame. When the coating has practically completely dried the surface thereof is moistened with water by 20 means of a sponge or a brush and the final coating 10 of gas resistant material, preferably in sheet form, is moistened and applied to the adhesive surface of the fabric by means of a roller. The coating material should be 25 rolled until all of the air bubbles are forced from between the gas resistant material and the surface of the fabric.

It will be observed that the initial coat of 30 cementing material is of a composition particularly adapted to adhere to the fabric while each successive coat of cementing material contains a smaller proportion of the substance capable of adhering to fabrics but a larger proportion of material adapted to adhere 35 here to the gas resistant film. This construction is highly important because it results in an excellent bond between the fabric and the gas resistant film even though there is no known cement adapted to adhere to both materials simultaneously.

Any suitable gas resistant substance may be 40 employed as a coating material. It has been observed by experience that the commercial cellulose derivative known as "cellophane" (a precipitated or regenerated cellulose xanthate), which may be obtained in the form of thin 45 transparent sheets of practically any desired size and thickness, is particularly suitable for the purpose. This material should be moistened with water containing about 5 percent glycerine before it is applied to the fabric.

In case it is desired to apply a gas resisting 50 film to an ordinary uncoated fabric, it is not necessary to employ latex containing solutions in order to obtain adhesion of the cementing material to the fabric. Instead, a 55 number of coats (preferably five or six) of a solution consisting of 40 grams of gelatin, 80 grams of glycerine, 1000 cc. of water and 2.4 60 grams of alum (a tanning agent) may be applied to the fabric and dried. The dried surface is then moistened with water by means of 65 a sponge or brush and the gas resistant film is

applied in the same manner employed in connection with rubberized fabric.

One of the extremely important features of the invention consists in drying the cementing film before the application thereto of the gas-resistant material, and this appears to be essential in order to obtain satisfactory results.

Materials prepared in accordance with the methods previously described have a high resistance to the diffusion of inflating gases. 75 They are also flexible and durable and the coating material adheres tenaciously to the surface of the fabric. The coating may also be protected by the application of additional coats of varnish or aluminum bronze or any 80 other desirable coating material, although the latter steps are not essential to the invention.

In addition to having excellent properties as gas retaining media, fabrics prepared in accordance with the method described may be 85 manufactured at relatively low cost, because sheet "cellophane", or equivalent materials, may be obtained at a small fraction of the initial cost of gold beater's skin of a quantity sufficient to coat a gas cell. Also, since the 90 materials may be obtained in relatively large sheets, one of which is sufficient to cover an entire width of fabric, it may be much more speedily and economically applied to the fabric than gold beater's skin. Furthermore, 95 these materials may be obtained in sheets that are practically uniform in character throughout, whereas gold beater's skin is likely to contain numerous small punctures difficult to detect. Fabrics coated with the former, therefore, require much less careful inspection 100 than fabric coated with gold beater's skin.

Although I have described in detail only the preferred embodiments of the invention, it will be apparent to those skilled in the art that it is not so limited, but that various minor modifications may be made therein without departing from the spirit of the invention or from the scope of the appended claims.

What I claim is:

1. A method of coating fabrics which comprises spreading thereon a film of cementing material adapted to adhere thereto, applying a second coating of cementing material adapted to adhere to a film of material having different adhesive properties from the fabric, drying the cementing materials, moistening the outer surface thereof and applying the film thereto.

2. A method of applying films of coating material to fabric which comprises coating the fabric with cementing material adapted to adhere thereto, applying successive coats of cement containing a material adapted to adhere to a film having different adhesive properties from the fabric, the proportion of the latter cementing material being progressively increased in succeeding coats, drying 130

the cementing coatings, moistening the surface thereof and applying the film thereto.

3. A method of applying gas-resistant materials to fabric which comprises coating the fabric with cementing material, drying the cementing material, moistening the surface and applying thereto a moistened sheet of gas-resistant material.

4. A method of coating fabrics with precipitated cellulose which comprises applying to the fabric a plurality of coatings of a cementing material, drying the cementing material, moistening the surface thereof and applying thereto a moistened sheet of cellulose.

10 5. A method of coating fabrics with sheets of regenerated cellulose which includes applying to the surface of the fabric successive coats of a gelatin solution, drying the coats, moistening the surface thereof and applying a coating of moistened cellulose material.

20 6. A method of applying cellulose films to rubber coated fabric which comprises coating the surface of the fabric with a suspension of rubber, applying additional coatings of a solution containing gelatin, drying the coatings, moistening the surface thereof and applying a sheet of cellulose material thereto.

25 7. A method of applying regenerated cellulose to fabrics which comprises coating the fabric with a cementing material, drying the cementing material, moistening the surface thereof and applying a sheet of moistened regenerated cellulose to the moistened surface.

35 8. A method of applying regenerated cellulose to rubberized fabrics which includes coating the fabric with an emulsion of rubber, applying to the latter coating a solution containing gelatin, allowing the gelatin coating to dry, moistening the surface thereof and applying thereto a film of moistened regenerated cellulose.

40 9. A method of manufacturing lighter-than-aircraft fabrics which comprises coating the fabric with a solution containing gelatin, drying the gelatin, moistening the surface thereof and applying thereto a film of a cellulose derivative.

45 10. A method of manufacturing lighter-than-aircraft fabrics which comprises coating the fabric with a solution containing gelatin, drying the gelatin, moistening the surface thereof and applying thereto a film of regenerated cellulose.

50 11. A balloon fabric having a plurality of coatings of a cementing material applied thereto, the inner layers of which consist essentially of rubber and the outer layers of which consist essentially of gelatin and an outer ply of regenerated cellulose adhering to the gelatin containing layers.

55 12. A balloon fabric having one coating consisting essentially of rubber, an additional coating consisting essentially of gela-

tin and a sheet of regenerated cellulose cemented to the latter coating.

In witness whereof, I have hereunto signed my name:

Signed at Evanston, in the county of Cook 70 and State of Illinois, this 29th day of November, 1927.

WILLIAM C. CALVERT.

75

80

85

90

95

100

105

110

115

120

125

130